

# UNITED STATES PATENT OFFICE.

CHARLES S. HALL, ADDISON B. CLEMENCE, AND H. F. AUGUST SETTERWALL,  
OF WORCESTER, MASSACHUSETTS.

## COATING FOR WIRE-DRAWING.

SPECIFICATION forming part of Letters Patent No. 339,168, dated April 6, 1886.

Application filed September 19, 1885. Serial No. 177,572. (No specimens.)

*To all whom it may concern:*

Be it known that we, CHARLES S. HALL, ADDISON B. CLEMENCE, and H. F. AUGUST SETTERWALL, all of the city and county of Worcester, and State of Massachusetts, have invented an Improved Coating for Wire Preparatory to Drawing, of which the following is a full, clear, and exact description, enabling others skilled in the art to which it applies to make and use the same.

In the manufacture of wire it is a well-known fact that the coating of said wire preparatory to drawing is a very important matter to be considered. A coating that will enable the accomplishment of certain desired results without at the same time involving any serious objections or disadvantages to the manufacturer is of great practical value, and has long been needed and sought for, much time and money having been expended in endeavors to improve the quality of coatings for the above purpose. Up to the present time, however, the coatings in use have not produced the most favorable results. While one coating may prove entirely satisfactory in one or more respects, its other objectionable features destroy said valuable qualities, and therefore results, as above stated, in an imperfect coating.

So far as we have been able to ascertain all of the present coatings in use embody the above objections in one form or another to a greater or less degree. One of the most serious objections is the thick pasty nature of some coatings, which it requires a long time to dry, and which also covers the wire unevenly, some places being thicker than others. It is obvious that such coatings require much more power in drawing the wire, and are also liable to absorb moisture after having been dried, therefore making it impossible to leave the unfinished wire on the blocks or reels over night without impairing the operation of drawing the same next day. Another objection to a coating of an absorbing nature is that it does not properly protect the wire covered by it from corrosion, some coatings

even hastening rather than retarding said corroding process.

The object of our invention is to obviate as far as is possible the foregoing objections to the present coatings.

It consists in immersing the wire, after having been cleaned in the usual way and preparatory to being drawn, in a solution of acetate of iron alone, or a mixture of acetate of iron and lime, meal, flour, or any other suitable and well-known lubricant in common use. We prefer in practice to use lime with the acetate of iron, as it dries the coating quicker, and aids in drawing the wire through the reducing-die.

The wire, having been cleaned in the usual way, as before stated, is next immersed or dipped in the solution of acetate of iron, or the same mixed with slaked lime or any of the other common, well-known lubricants, and then dried, after which it is ready to be drawn or reduced in size in the usual way.

In making the coating solution just sufficient water is added to the acetate of iron or other mixture to form a coating of the desired thickness upon the wire to properly draw the same. As it adheres well to the metal, it may be made very thin. It is deposited in a very uniform and smooth manner over the whole surface of the wire, and when dry forms a hard adhesive coating, which after the first draft through the reducing-dies is still further hardened to the consistency of cement. Therefore but little of the coating material is removed at each draft in the reducing process, which circumstance enables it to be drawn down one or more sizes smaller than by the use of the best of other known coatings.

By the use of our coating the wire may be drawn down until it becomes so brittle by reduction as to not admit of further reduction, a sufficient quantity of the coating material still remaining to properly protect the surface of said wire.

As the coating does not absorb moisture, it dries quickly, and will therefore not rust

the wire. It may be left for several days in a damp room upon the drawing-blocks or the floor with but little, if any, injury to its drawing qualities.

5 Having described our invention, what we claim therein as new, and desire to secure by Letters Patent, is—

1. A coating for wire, consisting of acetate of iron.

1c 2. A coating for wire-drawing, consisting

of acetate of iron and lime, meal, flour, or any other common well-known lubricant suitable for the purpose, substantially as described.

CHARLES S. HALL.  
ADDISON B. CLEMENCE.  
H. F. AUGUST SETTERWALL.

Witnesses:

ALBERT A. BARKER,  
LUCIUS W. BRIGGS.